

## UNITED STATES PATENT OFFICE

1,975,112

## BERYLLIUM ALLOY

Georg Masing, Berlin, and Otto Dahl, Berlin-Charlottenburg, Germany, assignors, by mesne assignments, to Metal & Thermit Corporation, New York, N. Y., a corporation of New Jersey

No Drawing. Application May 13, 1927, Serial No. 191,263. In Germany May 21, 1926

8 Claims. (Cl. 75—1)

The invention relates to alloys of beryllium with copper and phosphorus. The copper content of the new alloys preponderates over the beryllium content which preferably should be less than 5 per cent and at most amount to about 12 per cent, while the phosphorous content varies from a trace to about 1 per cent. In addition, other elements—for example tin, zinc and aluminium—may be present. By the presence of a little beryllium, copper is given new and valuable properties, including the possibility of being hardened to steel-like hardness. By the use of the stated other elements as auxiliaries, the new results may be obtained with a less proportion of beryllium.

15 Copper-beryllium alloys are of a yellowish, somewhat bronze like color or are somewhat paler and are characterized by great hardness, strength, and resistance to corrosion. They thus possess qualities that in certain circumstances considerably surpass those of the best bronzes and are somewhat similar to the properties of hardened steel. The alloys may be prepared, for example, by fusing together copper and beryllium, preferably after first alloying the beryllium with 25 another metal, with, if required, the addition of other elements such as tin, zinc, and aluminium. According to the invention an alloy of the aforesaid type is subjected in the solid state to a refining heat treatment.

30 As exhaustive experiments have shown, beryllium alone or in the presence of other metals is an excellent hardening agent for copper. In particular, it enables the properties of the prepared alloys of the above mentioned range of beryllium content to be improved by suitable thermic treatment, so that on the one hand the alloys can be put into a condition of sufficient softness and ductility for rendering them suitable for working by kneading and by cutting tools and, on the other hand, by means of another thermic treatment, some of these alloys can be given degrees of hardness surpassing that of hardened steel. By properly gauging the thermic treatment any required intermediate degree of hardness, 45 strength and toughness can be imparted. The alloys exhibit, in addition to good technological properties, a variability by thermic treatment to an extent hitherto unknown in other copper alloys.

50 The character of the thermic treatment depends upon the composition of the alloy and the purpose in view and will now be described. In the case of alloys containing up to about 5 per cent of beryllium the following thermic treatment is very advantageous:—the alloys are heated at

high temperatures, preferably above 600° C. and after sufficiently rapid cooling, by chilling in the case of large pieces and by cooling in the air in the case of small pieces, they are subjected to a second thermic treatment at lower temperatures, preferably between 150—500° C. The duration of the last mentioned thermic treatment depends primarily on the temperature; whereas in the neighbourhood of the lower temperature limit it may amount to several days, only two 60 hours will suffice at 300° C. and the time required becomes progressively shorter at higher temperatures. By means of this double heat treatment it is possible, for example, to raise the hardness of an alloy consisting of 97 per cent 70 of copper and 3 per cent of beryllium from about 125 to 360 Brinell units. The tempering effect of this heat treatment is also obtained in the case of a beryllium content above the aforesaid limit of 5 per cent but in the case of such higher percentages the tempering effect is so greatly overshadowed by other changes in the alloy as not to be directly appreciable; nevertheless, this heat treatment may be advantageous even in the case of these alloys for certain purposes which demand 75 the combination of a certain hardness and 80 tenacity.

While the tempering process hereinbefore described is applicable to all copper alloys containing up to about 10 per cent of beryllium, the 85 two processes now to be described are intended for use only with beryllium alloys of that type in which on solidification of the melt there first separates out a very hard  $\beta$ -crystal form which breaks down at a temperature below about 580° 90 C. Such are the alloys containing from 3—12 per cent of beryllium. By the addition of other elements, such as tin, zinc and aluminium, the concentration and temperature limits of the  $\beta$ -form are in their entirety shifted preponderatingly toward the side of the low beryllium content. In other words, the presence of the other elements permits the use of smaller amounts of beryllium in attaining the same results; they have an auxiliary action. It is evident that the range of applicability of the processes to be described extends in each of these cases over the range of existence of the  $\beta$ -crystals with reference to the changed 95 temperature relationships.

The object of the first of the two processes now 105 to be described is to impart a high degree of hardness to the alloy. For this purpose, the alloy is quenched from a temperature above the breaking down temperature of the  $\beta$ -crystals,—this in the case of the pure copper-beryllium alloys is 110

always above about 580° C. In this manner it is possible to impart, for example, a hardness of 730 to a copper-beryllium alloy with 6.7 per cent of beryllium which alloy originally has a hardness of 490 in the chilled casting.

If on the other hand it is required to obtain an alloy of this group in a workable condition, this is done by annealing at a temperature below that of the breaking down of the  $\beta$ -crystals—thus, in the case of the pure copper-beryllium alloy, below 580° C.—and so completely breaking down the  $\beta$ -crystals and obtaining the alloy in a comparatively soft condition; its hardness in the case of a 6.7 per cent beryllium content will thus be brought to about 240.

As already stated, the last mentioned process may be combined with the first mentioned thermic treatment.

The various thermic treatments described may be applied to cast as well as to worked alloys.

If it be desired to obtain copper-beryllium alloys having a high ductility and toughness in addition to considerable strength we may proceed as follows:—

The alloy is, after a preliminary mechanical treatment (working, as by hammering, rolling, etc.) or chemical treatment, if such preliminary treatment be required, heated to temperatures below those given for the first heating—for example, below 600° C.—but above the temperatures of the second heating—for example, above 450° C. The alloys can also be heated for a rather long time at somewhat lower temperatures at which practically only a hardening effect is produced which, however, on longer heating is replaced by a high ductility and toughness in addition to considerable strength. As the heating can be interrupted at any suitable moment it is possible in this way to produce, as desired, alloys having within wide limits definite values for hardness, ductility, toughness and strength.

Practically identical with the heat treatment described is one in which the alloy is heated at a temperature higher than 600° C. and then slowly cooled.

For example, a copper-beryllium alloy containing 2.5 per cent of beryllium is heated at 500° C. and thus acquires a notched bar test toughness of about 15 meter kilograms per square centimeter with a strength of over 75 kilograms per square millimeter, while the same alloy after being thermally treated as above described by being heated twice at different temperatures—for example, above 600° C. and up to about 450° C.—exhibited a notched bar test toughness of only 1 meter kilogram per square centimeter with a strength of 140 kilograms per square millimeter.

It has been discovered in this connection that substantial results are obtained with the single heating process only when the beryllium content of the alloy amounts to at least 1 per cent.

It has further been discovered that very valuable properties can be imparted to a copper-beryllium alloy with a low beryllium content by the addition of up to 1 per cent of phosphorus. The thermic tempering process of the copper-beryllium alloy is accelerated by the phosphorus content and, moreover, a considerable improvement of the properties is effected by this thermic treatment even in the case of a low beryllium content, so that the addition of phosphorus at the same time renders possible a saving in costly metallic beryllium; in this case one or more other elements—for example, zinc, tin, alumin-

ium, and magnesium—may also be present in the alloy.

The thermic treatment of a copper-beryllium alloy containing phosphorus is carried out, for example, as follows:—

An alloy containing about 0.25 per cent of phosphorus and about 1.50 per cent of beryllium was heated at about 800° C. and then quickly cooled. After cooling, its hardness amounted to about 80 units. By then heating the alloy for an hour at 350° C. the hardness was increased to 210 units. When, on the other hand, a copper-beryllium alloy with the same beryllium content but free from phosphorus was subjected to a corresponding thermic treatment, the hardness, after rapidly cooling the alloy from 800° C., amounted to 74 units and even on heating the alloy for seven hours in this case the hardness rose only by about 20 units. From this example the considerable improvement of the alloy by the addition of phosphorus is clearly evident.

After the above described copper-beryllium-phosphorus alloys have been subjected to one or more of the above mentioned tempering heat treatments, they are very suitable for use as material for metallic springs, for example as leaf, helical, or spiral springs as well as for parts of machinery or apparatus that are subjected to friction, especially axle bearings, commutators, sliding contacts, or other electric current conducting members.

By the expression "balance substantially copper" found in the accompanying claims we mean that the alloys called for may contain small quantities of addition metals, such as aluminum, tin, silver, magnesium and zinc in proportions insufficient to substantially change the characteristics of the said alloys.

What we claim as our invention and desire to secure by Letters Patent is:

1. An alloy characterized by hardness, strength and resistance to corrosion, containing from about 0.3 to 12 per cent of beryllium and from about 0.1 to 1 per cent of phosphorus, with a remainder substantially copper.

2. An alloy characterized by hardness, strength and resistance to corrosion, containing from about 3 to 12 per cent of beryllium and from a trace to about 1 per cent of phosphorus with a remainder substantially copper.

3. An alloy characterized by hardness, strength and resistance to corrosion, containing from about 0.3 to 12 per cent of beryllium, a phosphorus content of from about 0.1 to 1 per cent and also containing from about 0.1 to 8 per cent of aluminum, with a remainder substantially copper.

4. An alloy characterized by hardness, strength and resistance to corrosion, containing from about 3 to 12 per cent of beryllium, a phosphorus content varying from a trace to about 1 per cent and also containing from about 0.1 to 8 per cent of aluminum, with a remainder substantially copper.

5. An alloy characterized by hardness, strength and resistance to corrosion, containing from about 0.3 to 12 per cent of beryllium, a phosphorus content of from about 0.1 to 1 per cent and also containing from about 0.1 to 8 per cent of tin, with a remainder substantially copper.

6. An alloy characterized by hardness, strength and resistance to corrosion, containing from about 3 to 12 per cent of beryllium, a phosphorus content varying from a trace to about 1 per cent

and also containing from about 0.1 to 8 per cent of tin, with a remainder substantially copper.

7. An alloy characterized by hardness, strength and resistance to corrosion, containing from about 0.3 to 12 per cent of beryllium, a phosphorus content of from about 0.1 to 1 per cent and also containing from about 0.1 to 8 per cent of zinc, with a remainder substantially copper.

8. An alloy characterized by hardness, strength and resistance to corrosion, containing from about 3 to 12 per cent of beryllium, a phosphorus content varying from a trace to about 1 per cent and also containing from about 0.1 to 8 per cent of zinc, with a remainder substantially copper. 80

GEORG MASING.  
OTTO DAHL.

10

85

15

90

20

95

25

100

30

105

35

110

40

115

45

120

50

125

55

130

60

135

65

140

70

145

75

150